

I. G. JOHNSON.  
MERCURY BOTTLE.

No. 21,835.

Patented Oct. 19, 1858.

*Fig. 1.*



*Fig. 2.*



# UNITED STATES PATENT OFFICE.

ISAAC G. JOHNSON, OF SPUYTEN DUYVIL, NEW YORK.

## IMPROVEMENT IN BOTTLES FOR CONTAINING MERCURY.

Specification forming part of Letters Patent No. 21,835, dated October 19, 1858.

*To all whom it may concern:*

Be it known that I, ISAAC G. JOHNSON, of Spuyten Duyvil, in the county of Westchester and State of New York, have invented or discovered a certain new and useful Bottle for Containing Mercury for Transportation and other Purposes; and I do hereby describe and ascertain the same, referring to the accompanying drawings, in which—

Figure 1 is an exterior view; Fig. 2, a section.

Heretofore the bottles used in commerce for holding mercury or quicksilver have been made of wrought-iron. This was the only material that was sufficiently strong and secure for the purpose. Cast-iron would have been too liable to break and too porous to contain it with safety, and greatly increased the weight over wrought-iron. Other metals would be amalgamated, and glass, pottery, &c., are too fragile. The wrought-iron bottles are seamed on the side, and will sometimes open on receiving a heavy blow—such as they are liable to—and are exceedingly expensive, so much so, in fact, as to preclude the manufacture in the United States, as far as I know. I have devised a bottle at once as light and portable as the wrought-iron, and as strong and safe in every particular, if not more sure not to leak under the roughest usage.

My bottle is made of malleable cast-iron, as follows: I make a pattern of the desired form, from which the exterior is molded; but instead of so forming the core as to vent only at the top through the neck, I pass a center vent or core clear through, leaving a small hole through the bottom of the bottle. This mode of making the

core has several advantages: First, it gives more perfect and freer vent, preventing a porous casting or "blows" therein; and, secondly, it enables me to make the casting thinner and lighter than could otherwise be done, and more fully insures the equal thickness of the sides of the bottle. The bottle thus cast is filled with carefully-prepared decarbonizing compound, with which it is also surrounded, and is then submitted to a heated annealing furnace in the usual way. It will be noted that if there is an opening in both ends of this bottle it admits of a current through it and a free escape for gases. These several advantages are necessary to obtain the most perfect results in annealing and manufacturing. After the bottle is made and perfectly annealed it is finished by inserting a plug in the bottom and welding it tight, or otherwise fastening it so as to be mercury-tight. A bottle thus made I have put to the severest tests with perfect safety. It can readily be beaten flat, so as to collapse both sides together without injury, and a fall of any distance to which the bottle in practice would be liable would do no injury or endanger its contents.

Having thus fully described my improved mercury-bottle, what I claim is—

The mercury-bottle formed and composed of malleable cast-iron, substantially in the manner and for the purpose set forth.

In testimony whereof I have hereto set my hand this 21st day of July, 1858.

ISAAC G. JOHNSON.

In presence of—

HENRY STANLEY,  
W. WEBB.